# EUROPEAN PATENT SPECIFICATION

(11) **EP 0 041 984 B1**
(45) Date of publication and mention of the grant of the patent: **19.09.1984**
(21) Application number: 81900099.3
(22) Date of filing: 27.10.1980
(51) Int. Cl.: G03C 1/60, G03C 1/54, G03C 1/72

(54) **DIAZONIUM IMAGING SYSTEM**
DIAZOPHOTOGRAPHISCHES SYSTEM
SYSTEME PHOTOGRAPHIQUE AU DIAZONIUM

(30) Priority: 07.12.1979 US 101143
(43) Date of publication of application: 23.12.1981
(73) Proprietor: MINNESOTA MINING AND MANUFACTURING COMPANY, St. Paul, Minnesota 55133-3427 (US)
(72) Inventor: GATZKE, Kenneth G., St. Paul, MN 55133 (US)
(74) Representative: Baillie, Iain Cameron
(86) International application number: US8001444
(87) International publication number: WO8101756

## Description

### 1. Field of the Invention

A novel light sensitive, heat developable imaging system incorporating a diazonium salt and a leuco dye in a binder is disclosed. The system is useful, for example, as a microfilm duplicating sheet or a heat sensitive recording material.

### 2. Description of the Prior Art

U.S. Patent 3,390,997 discloses a light-sensitive admixture of an alkylthio, benzylthio, 2-phenyl- hydrazino or alkoxycarbonyl derivative of a triphenylmethane compound (a "leuco dye") and a selected non-volatile nitrogen-containing compound which functions as a photooxidant useful as an imaging system. The light sensitive compounds ofthe present invention differ significantly from those of the patent which contain only trivalent nitrogen atoms. Furthermore, the present invention requires elevated temperatures 82°C to 193°C [180°F to 380°F] for image development, whereas the patent disclosure is of a room temperature developing system.

U.S. Patent 3,445,233 relates to a composition which may contain a polymeric binder in addition to three active ingredients which are an organic nitrogen-containing color generator, a photooxidant, and diazonium_{'} compound. The photooxidant oxidizes the color generator in the presence of radiation. There is no reaction between the color generator and the diazonium salt when irradiated.

An imaging system comprising a leuco dye, a diazonium salt, and nitrate ion in a binder is described in assignee's copending patent application, International Publication No. WO 81/01757 (European Patent Application No. 81 900104.1) published 25 Jun 1981. This four-part imaging system does not suggest the efficacy of the three-part imaging.

An imaging system comprising a polymeric binder, a bleachable dye or leuco dye, a photosensitive diazonium salt, and at least 0.1 mole nitrate ion/1.0 mole dye is described in assignee's copending patent application, International Publication No. WO 81/01755 (European Patent Application No. 81 900 234.6) published 25 June 1981.

### Disclosure of the Invention

The present invention relates to a light sensitive, heat developable imaging system comprising a polymeric binder resin, a leuco dye, and a diazonium salt. In the practice of the present invention the chemical nature of the polymer including its acid content has not been found to be a functional requirement. However, it is preferred to have an acid present (e.g., organic or inorganic acid) in the coating composition. Preferably, the acid is present in at least equimolar proportions to the diazonium salt.

Furthermore, no oxidizing anion, including nitrate ion, is a necessary component of the present invention as it is in assignee's copending application mentioned above. If any nitrate ion is present, it is in amounts of less than 0.1 mole nitrate/1.0 mole dye. Other oxidizing anions and compounds may be present in greater or lesser amounts, but are not essential in the practice of the present invention.

In the present invention, the leuco dye (a clear to faintly colored material), the diazonium salt and the polymeric binder resin are incorporated in a solvent system and cast on any substrate such as paper, polymeric filmn such as polyester, glass, metal, ceramics and the like. Upon irradiation by light, the diazonium salt is destroyed. The subsequent application of heat to the coating results in oxidation of the leuco dye by the diazonium salt to a colored form in the non-light struct portion of the coating. A positive-acting image is thus produced since color is generated where no light has contacted the coating.

Although the precise mechanism of the image formation is not understood, as mentioned above the reaction appears to be an oxidation of the leuco dye during heat development by the diazonium salt which has not been decomposed by incident radiation.

### Detailed Description of the Invention

The present invention provides a light-sensitive, positive-acting, heat developable layer on a substrate, said layer comprising a polymeric binder, a leuco dye, and a diazonium salt, the dry ingredients of said layer characterized by including at least 25 percent by weight of a polymeric binder, at least 0.3 percent by weight of a leuco dye capable of being oxidized to a colored form, a sufficient amount of a photosensitive diazonium salt to oxidize said leuco dye, upon heating, to a colored form in non-light struck portions of said layer, and less than 0.1 mole nitrate ion per 1.0 mole leuco dye.

### The Binder

Any natural or synthetic polymeric binder may be used in the practice of the present invention. Organic polymeric resins, preferably thermoplastic resins (although thermoset resins may be used), are generally preferred. The most preferred resins are polyvinyl acetate and polyvinyl chloride copolymers. Such resins as polyvinyl acetals, polyesters, polyvinyl resins, polyvinylpyrrolidone, polyesters, polycarbonates, polyamides, polyvinyl butyral, polyacryllates, cellulose esters, copolymers and blends of these classes of resins, and others have been used with particular success. Natural polymeric materials_{'} such as gelatin and gum arabic may also be used. Where the proportions and activities of the leuco dye and diazonium salt require a particular developing time and temperature, the resin should be able to withstand those conditions. Generally it is preferred that the polymer not decompose or lose its structural integrity at (147°C) (300°F) for 60 seconds and most preferred that it not decompose or lose its structural integrity at (193°C) (380°F) for 5 minutes. Also, polymers must be compatible with the other components and solvents, in addition to having a reasonably low softening point for processability. Such polymers desirably are permeable to trapped gases.

In addition to these requirements, the selected binder must be transparent or translucent and be either clear or lightly colored. This will ensure an obvious contrast with colored areas (non-light struck) after heat development.

The binder may serve a number of additionally important purposes in the constructions of the present invention. The imageable materials may be protected from ambient conditions such as moisture. The consistency of the coating and its image quality are improved. The durability of the final image is also significantly improved. The binder should be present as at least 25% by weight of ingredients in the layer, more preferably as at least 50% by weight and most preferably as at least 70% by weight of dry ingredients (i.e., excluding solvents in the layer).

### Dyes

Leuco dyes are well known in the art. These are colorless or lightly colored dyes which when subjected to an oxidation reaction form a colored dye. These leuco dyes are described in the literature (e.g., Mees and James, "The Theory of the Photographic Process", 3rd Edition, published 1966, by Macmillan Co. (N.Y.), see pages 283-4, 390-1; and J. Kosar, "Light-Sensitive Systems", published 1 d65, by Wiley and Sons, Inc. (N.Y.), see pages 367, 370-380, 406). Amongst the best known leuco dyes are leuco crystal violet (LCV) and Leuco malachite green (LMG). Only those leuco dyes which can be converted to colored dyes by oxidation are useful in the practice of the present invention. Acid or base sensitive dyes such as phenolphthalein and other indicator dyes are not useful in the present invention unless they are also oxidizable to a colored state. Indicator dyes would only form transient images or would be too sensitive to changes in the environment. The leuco dyes which have been specifically shown to work in the present invention are discussed in detail below, including their formulae; and include but are not limited to the following:
Leuco Crystal Violet (available in leuco form from Fisher Scientific Co., Pittsburg, PA) (oxidized form is C142555) Leuco Malachite Green (available in leuco form from Fischer Scientific Co.) (oxidized form is CI 42000) Copikem II (Hilton Davis, Div. of Sterling Drug, Inc., Cincinnati, OH) Leuco Atacyl Orange-LCM (dye form available from Atlantic Chemical Corp., Mutley, NJ) Leuco Atacryl Brilliant Red-4G (dye form available from Atlantic Chemical Corp.) Leuco Ethyl Violet (dye form CI 42600, available from Fischer Scientific Co.) Leuco Victoria Blue-BGO (dye form CI 42595, available from Dye Specialities, Inc., Seacaucus, NJ) Leuco Atacryl Yellow-R (dye form available from Atlantic Chemical Corp.) Leuco Atlantic Fuchsine Crude (dye form CI 42500, available from Atlantic Chemical Corp.)

The leuco dyes of the present invention become colored due to oxidation, that is, they have absorbance after coloration in the visible portion of the electromagnetic spectrum (approximately 400 to 700 nm). The leuco dye should be present as at least 0.3% by weight of the binder layer, preferably at least 1 % by weight, and mist preferably at least 2% to 10% or more by weight of the dry weight of the imageable layer.

In forming the leuco dye layer or coating of the dye layer onto a substrate, temperatures should, of course, not be used during manufacture which would colorize the layer or decompose the diazonium salts. Some slight colorization is tolerable, with the initial leuco dye concentrations chosen so as to allow for anticipated colorization. It is preferred, however, that little or no leuco dye be colorized during forming or coating so that more standardized layers can be formed. Depending on the anticipated development temperature, the coating or forming temperature can be varied. Therefore, if the anticipated development temperature were, for example, 167°C, the drying temperature could be 138°C, and it would not be desirable for the layer to gain 20% of its optical density at the drying temperature in less than 4-5 minutes. Such a gain would be tolerable by correspondingly increasing the amount of leuco dye.

There should be sufficient colorizable dye present in the colorizable layer of the present invention to provide an increase in optical density upon development of at least 0.2, more preferably 0.6, and most preferably 1.0 or greater. These increases can be measured at the development temperatures for the imaging materials, e.g., 132°C for 60 seconds. Thus the preferred limitation of at least 0.2 gain in optical density or absorbance of colorless light at 132°C for 60 seconds is based on the assumption of a development temperature of 132°C. For an anticipated higher or lower development temperature, the 0.2 gain in optical density or absorbance should occur at that development temperature within a reasonable period of time. A reasonable development temperature range is between 82°C and 193°C and a resonable dwell time is between 5 seconds and 5 minutes, preferably at between 105°C and 167°C and for 10 to 180 seconds, with the longer times most likely accosicated with the lower development temperatures. Therefore, all of the absorbance characteristics are applicable to the generally useful development range of 82°C to 193°C.

### Diazonium Salts

Light sensitive diazonium salts are well known in the art. These salts comprise a light sensitive aromatic nucleus with an external diazonium group and an anion associated therewith (e.g., J. Kosar, "Light-Sensitive System", published 1965, by John Wiley and Sons, Inc. (N.Y.), see pages 202-214; and P. Glafkides, "Photographic Chemistry", Vol. II, published 1960, by Fountain Press (London), see pages 709-725). They may be generally represented by the formula:

### wherein Ar is an aromatic nucleus, and X- is an anion.

Any anion may be used in the diazonium salt. Anions as diverse as zinc chloride, tri-isopropyl naphthalene sulfonate, fluoroborate (i.e., BF4-), and bis(perfluoroalkylsulonyl)methides may be used. The change in anions may affect the speed of the imaging layer, but not its function. Any light sensitive aromatic diazonium nucleus, as known in the art, may also be used in the practice of the present invention. These diazonium nuclei, particularly those belonging to the classes pyrrolidine, morpholine, aniline, and diphenyl amine and its polymers are well known in the art and include, for example, P-anilinobenzene; N-(4-diazo-2,4-dimethoxy phenyl)pyrrolidine; 1-diazo-2,4-diethoxy-4-morpholino benzene; 1-diazo-4-benzoyl amino-2,5-diethoxy benzene; 4-diazo-2,5-dibutoxy phenyl morpholino; 4-diazo-1-dimethyl aniline; 1-diazo-N,N-dimethyl aniline; 1-diazo-4-N-methyl-N-hydroxyethyl aniline; etc.

### Additives

Other materials which may be useful in the formulations of the present invention include reducers and complexors, plasticizers and polyketones, stabilizers, surfactants, antistatic agents, coating aids, oxidizing materials (other than nitrate ion which may be present only in amounts less than 0.1 mole nitrate to 1.0 mole dye), inhibitors, lubricants, flexibilizers, fillers and the like.

All of this will be more thoroughly understood by consideration of the following examples:

### Examples 1-11

These examples examine the effect of using different binders in the formulation. Two separate solutions, A and B, are prepared. Solution A comprised .020 g phthalic acid, .010 g catechol, .10 g Phenidone A (1-phenyl-3-pyrazolidone), .200 g aromatic ketone resin, .200 g polymeric plasticizer (ter, 2,4-trimethylpentane, 1,3-diol adipate 2-ethylhexanol terminated [900-1100 molecular weight]) and 1.060 g methyl ethyl ketone (MEK) for a total weight of 1.5 g. Solution B comprised .051 g leuco crystal violet (4,4',4"-methylidynetris-(N-N-dimethylaniline)), .046 g leuco malachite green (p,p'- benzylidenebis-(N,N-dimethylaniline)), and 1.429 g tetrahydrofuran (THF), for a total weight of 1.5 g. 1.5 g of each of solutions A and B were mixed with 0.1 g 1-diazo-2,5-diethoxy-4-morpholino benzene borofluoride DDMBB) and in each case with the stated amount(s) of binder(s), (see Table 1), to form a solution which was then coated on polyethylene terephthalate film to a thickness as noted in the table. The coated film was dried at 71 °C, exposed to a mercury vapor lamp for 10⁶ meter-candle-seconds, and then developed for 60 seconds at 132°C. The optical densities in the light struck (LS) areas, also referred to as Dmin, and the non-light struck (NLS) areas, also referred to as Dmax, are recorded in Table 1.

Phthalic acid is useful in these formulations to stabilize the coating solution by preventing the diazonium salt from reacting before development.

The change in optical density (ADensity), i.e., Dmax-Dmin, is of great significance and values in excess of 1.0 are of commercial practicability. Examples 6 and 11 show the greatest changes in optical density (Dmax-Dmin) between light struck and non-light struck areas. It appears, therefore, that vinyl acetate and vinyl chloride copolymers, VC-VA-87/13-1 and VC-VA-VAL-91/3/5.7, are the preferred resins in the practice of this invention.

### Examples 12-19

These examples further investigate vinyl chloride and vinyl acetate binders. The reference solution (1.5 g each of solutions A and B, and 0.1 g DDMBB) was prepared and mixed with the stated amount of binder (Table 2), then coated and treated as in examples 1-11. Results appear below.

The binders of examples 12, 13 and 14 decrease progressively in molecular weight which correlates with a progressive decrease in softening points of these resins. It is of note that the A Density increases as the softening temperature of the resin decreases, reflecting better reacting conditions in softer resins.

The binders of examples 15 and 16 are resins with acid content, a factor which did not enhance the A Density.

The resins of example 14 (lo /ter molecular weight) and example 17 (hydrolyzed) provided the best A Density of those tested in this group.

### Examples 20-33

The following acids and a control were screened with the resin of example 14 (VC-VA 87/13-2) using in each case 0.1 g DDMBB and 4.0 g of a master batch solution comprising 2.0 g LCV, 18.0 g toluene and a solution containing 60.0 g of 40% VC-VA-87/13-2, 18% MIBK, 18% ethanol and 24% MEK:

Although the most common effect appeared to be a reduction in both optical densities, Dmin and Dmax, the opposite was also true in some cases. Only nitric acid appeared to increase the maximum density and reduce the minimum density by stabilizing the diazo and also aiding in the oxidation of the leuco dye. This is an example of the effect of nitrate ion in the formulation and is the subject of assignee's copending application mentioned above. In sum, the non-nitrate acid content of the formulation has not been found to be a significant factor in the practice of this invention.

### Examples 34-52

In a search for materials which would lower the Dmin and increase the Dmax, tests were performed on the addition of small amounts (.05 g) of various reducers and complexors (antioxidants or chelating agents) in a solution of .01 g DDMBB and .85 g 1:1 methanol and acetone added to portions of a master batch comprising 2.2 g leuco crystal violet, 19.8 g toluene and 66.0 g of a solution containing 40% VC-VA-87/13-2, 10% methyl isobutyl ketone, and 50% methyl ethyl ketone. The materials tested were:

Tetrachlorophthalic anhydride, 2,4,4-trimethylpentyl-bis-(2-hydroxy-3,5-dimethylphenyl)methane (TBHDM), 2,6-bis(2'-hydroxy-3'-tert butyl-5'-methyl benzyl)-4-methylphenol, and 2,2'-methylenebis(4-methyl-6-tert butylphenol) showed some degree of usefulness in increasing the A Density compared to experiments without these materials. Phenidone A (1-phenyl-3-pyrazolidone) and ascorbic acid greatly depressed both the Dmin and Dmax values and when studied at lower levels of concentration (.01 g) were found to be useful in depressing the Dmin.

### Examples 53-68

Small amounts of various polyketones, plasticizers, metal salts, and benzoyl peroxide were screened for their possible effect in lowering the softening point of the resin using 4 g of a master batch solution comprising 2.0 g leuco crystal violet, 18.0 g toluene, and 60.0 g of a solution containing 40% VC-VA-87/13-2, 18% methyl isobutyl ketone, 18% ethanol, and 24% methyl ethyl ketone. 0.1 g DDMBB dissolved in less than 1.0 g of 1:1 methyl alcohol and acetone was added. The materials tested were:

The results of these tests showed no dramatic improvement in A Density. It was found that plasticisers and polyketones effectively lower the softening point of the polymeric binder, thereby increasing the rate of development. They have been found to be most effective in the higher softening resins (i.e. resins of higher molecular weight) as might be expected.

### Examples 69-97

These examples tested the effect of variations in the diazonium salts. Using 4 g of the same master batch just described a study was made of the effect of the following 29 diazonium salts on the A Density, .1 g diazonium salt being dissolved in .9 g of a solution of 50% methanol and 50% acetone.

All of the diazonium salts proved useful in producing an image except p-nitrobenzene diazonium borofluoride which was very unstable and reacted prematurely in solution. Tests including diphenylamine-4-diazonium borofluoride (DDBF), 1-diazo-2,5-diethoxy-4-morpholino benzene borofluoride and 2,5-diethoxy-4-(p-tolyethio)benzene diazonium chloride 1/2 zinc chloride gave the highest Dmax values but the A Density values were not improved due to corresponding higher Dmin values.

### Examples 98-127

A study was made of the most effective compounds from previous examples. A diazo solution containing 2.5 g DDBF (diphenylamine-4-diazonium borofluoride) and 22.5 g of 50% methanol/50% acetone was prepared. Also Master Batch #1 (1.6 g leuco crystal violet, 14.4 g toluene and 48.0 g of a solution containing 40% VC-VA-87/13-2 dissolved in 10% MIBK/50% MEK) and Master Batch #2 (0.8 g leuco crystal violet, 15.2 g toluene, and 48.0 g of solution containing 40% VC-VA-87/13-2 dissolved in 10% MIBK/50% MEK) were prepared. The materials listed below were also tested using 1.0 g diazo solution in 4.0 g Master Batch #1, and they were tested using 0.5 g diazo solution in 4.0 g Master Batch _{#}2.

1,1,2-trimethyl-5-carboxyl-3-(p-carboxyphenyllindan (TCCI) and TBHDM were found to be effective in reducing the Dmin and thereby increasing the A Density values to some extent.

### Examples 128-129

Analysis of formulations containing variable amounts of Phenidone A, phthalic acid, 1:1 DDMBB and DDBF, leuco crystal violet, TCCI, ascorbic acid, and a solution of 40% VC-VA-87/13-2 dissolved in 10% MIBK/50% MEK, in addition to solvents, was made. The best results were obtained from formulations of examples 128 and 129, shown below in Table 3.

### Examples 130-139

These examples examine variations of the "best formulations" from the previous tests. Results are tabulated in Table 4. Initial density (D,) refers to the optical density of the coating before exposure to light and heat and as noted previously Dmin refers to the optical density of the light struck areas after exposure to light and heat and Dmax refers to the optical density of the non-light struck area after exposure to light and heat.

Examples 130, 131, 135 and 139 gave borderline commercial results, the Density values being respectively 1.16, 1.00, 1.02 and .94. The resolution in these cases is excellent, being in the order of 400 line pairs per mm.

Additional experiments were run to test the effects upon the image produced by varying leuco dyes in the formulations. Leuco crystal violet and leuco malachite green were the most effective dyes in the practice of this invention. All the dyes tested and listed below were found to have utility in the present invention but the formulations must be optimized to make a useful product.

1) Leuco Crystal Violet 4,4',4"-methylidynetris-(N,N-dimethylaniline)
.2) Leuco Malachite Green p-p'benzylidenebis-(N,N-dimethylaniline)
3) Copichem II
4) Leuco Atacryl Orange-LGM: Color Indes Basic Orange 21, Comp. _{#}48035 (a Fischer's base type compound)
5) Leuco Atacryl Brilliant Red -4G: Color Index Basic Red 14
6) Leuco Ethyl Violet: Color Index Basic Violet 4, comp. #42600
7) Leuco Victoria Blue - BGO: Color Index Basic Blue 728 a, comp. _{#}44040
8) Leuco Atacryl Yellow ― R Color Index Basic Yellow 11, Comp. _{#}48055
9) Leuco Atlantic Fuchsine Crude:

## Claims

1. A light sensitive, positive-acting, image-forming layer on a substrate, said layer comprising a polymeric binder, a leuco dye, and a diazonium salt, the dry ingredients of said layer characterized by being heat developable and including at least 25% by weight of a polymeric binder, at least 0.3% by weight of a leuco dye capable of being oxidized to a colored form, a sufficient amount of a photosensitive diazonium salt to oxidize said leuco dye, upon heating, to a colored form in non-light struck portions of said layer, and less than 0.1 mole nitrate ion per 1.0 mole leuco dye.

2. The layer according to claim 1 further characterized by the feature that said leuco dye comprises in the range of 1 % to 10% by weight of dry ingredients of said layer.

3. The layer according to any preceding claim characterized by the feature that said leuco dye is present in a concentration sufficient to provide an increase in optical density upon development of at least 0.2.

4. The layer according to any preceding claim characterized by the feature that said leuco dye is present in a concentration sufficient to provide an increase in optical density upon development of at least 0.6.

5. The layer according to any preceding claim characterized by the feature that said leuco dye is present in a concentration sufficient to provide an increase in optical density upon development of at least 1.0.

6. The layer according to any preceding claim characterized by the feature that said leuco dye is selected from the class consisting of leuco crystal violet and leuco malachite green.

7. The layer according to any preceding claim characterized by the feature that said layer comprises the diazonium salt 1-diazo-2,5-diethoxy-4-morpholino benzene borofluoride.

8. The layer according to any preceding claim characterized by the feature that said layer comprises a binder selected from the classes consisting of polyvinyl chloride and polyvinyl acetate resins.

9. The layer according to any preceding claim characterized by the feature that said binder is present as at least 25% by weight of dry ingredients in the layer.

## Revendications

1. Une couche photographique positive photosensible sur un substrat, ladite couche comprenant un liant polymère, un colorant leuco et un sel de diazonium, les ingrédients secs de ladite couche étant caractérisés en ce qu'ils sont développables par la chaleur et comprennent au moins 25% en poids d'un liant polymère, au moins 0,3% en poids d'un colorant leuco pouvant être oxydé en une forme colorée, une quantité d'un sel de diazonium photosensible suffisante pour oxyder ledit colorant leuco par chauffage en une forme colorée dans les portions non frappées par la lumière de ladite couche et moins de 0,1 mole d'ion nitrate pour 1,0 mole de colorant leuco.

2. La couche selon la revendication 1, caractérisée de plus par le fait que la quantité dudit colorant leuco est comprise dans la gamme de 1% à 10% du poids des ingrédients secs de ladite couche.

3. La couche selon l'une quelconque des revendications précédentes, caractérisée par le fait que ledit colorant leuco est présent à une concentration suffisante pour réaliser un accroissement de la densité optique après développement d'au moins 0,2.

4. La couche selon l'une quelconque des revendications précédentes, caractérisée par le fait que ledit colorant leuco est présent à une concentration suffisante pour réaliser un accroissement de la densité optique après développement d'au moins 0,6.

5. La couche selon l'une quelconque des revendications précédentes, caractérisée par le fait que ledit colorant leuco est présent à une concentration suffisante pour réaliser un accroissement de la densité optique après développement d'au moins 1,0.

6. La couche selon l'une quelconque des revendications précédentes, caractérisée par le fait que ledit colorant leuco est choisi parmi la catégorie constituée par la forme leuco du cristal violet et la forme leuco du vert malachite.

7. La couche selon l'une quelconque des revendications précédentes, caractérisée par le fait que ladite couche comprend le sel de diazonium 1-diazo-2, 5-diéthoxy-4-morpholino-benzène borofluorure.

8. La couche selon l'une quelconque des revendications précédentes, caractérisée par le fait que ladite couche comprend un liant choisi dans les catégories constituées par les résines de chlorure de polyvinyle et les résines d'acétate de polyvinyle.

9. La couche selon l'une quelconque des revendications précédentes, caractérisée par le fait que ledit liant est présent à raison d'au moins 25% du poids des ingrédients secs de la couche.

## Patentansprüche

Positivwirkende lichtempfindliche Bilddarstellungsschicht auf einem Substrat, wobei die genannte Schicht ein polymeres Bindemittel, einen Leukofarbstoff und ein Diazoniumsalz enthält und die Trockenbestandteile der Schicht dadurch gekennzeichnet sind, daß sie in der Wärme entwickelbar sind und mindestens 25 Gew.% eines polymeren Bindemittels, mindestens 0,3 Gew.% eines in einen farbigen Zustand oxidierbaren Leukofarbstoffes, eine bei Erwärmung zum Oxidieren des Leukofarbstoffes in nicht lichtbeaufschlagten Teilen der Schicht genügende Menge eines lichtempfindlichen Diazoniumsalzes und weniger als 0,1 Mol Nitration pro 1,0 Mol Leukofarbstoff enthalten.

2. Schicht nach Anspruch 1, dadurch gekennzeichnet, daß der Leukofarbstoff 1 bis 10 Gew.% der Trockenbestandteile der genannten Schicht ausmacht.

3. Schicht nach einem der vorhergehenden Ansprüche, dadurch gekennzeichnet, daß der Leukofarbstoff in einer so hohen Konzentration vorhanden ist, daß er bei seiner Entwicklung die optische Dichte um mindestens 0,2 erhöht.

4. Schicht nach einem der vorhergehenden Ansprüche, dadurch gekennzeichnet, daß der Leukofarbstoff in einer so hohen Konzentration vorhanden ist, daß er bei seiner Entwicklung die optische Dichte um mindestens 0,6 erhöht.

5. Schicht nach einem der vorhergehenden Ansprüche, dadurch gekennzeichnet, daß der Leukofarbstoff in einer so hohen Konzentration vorhanden ist, daß er bei seiner Entwicklung die optische Dichte um mindestens 1,0 erhöht.

6. Schicht nach einem der vorhergehenden Ansprüche, dadurch gekennzeichnet, daß der Leukofarbstoff aus der Klasse ausgewählt ist, die aus Leukokristallviolett und Leukomalachitgrün besteht.

7. Schicht nach einem der vorhergehenden Ansprüche, dadurch gekennzeichnet, daß sie das Diazoniumsalz 1-Diazo-2,5-diethoxy-4-morpholinobenzolborfluorid enthält.

8. Schicht nach einem der vorhergehenden Ansprüche, dadurch gekennzeichnet, daß sie ein Bindemittel enthält, daß aus den Klassen ausgewählt ist, die aus den polyvinylchlorid- bzw. den Polyvinylacetatharzen bestehen.

9. Schicht nach einem der vorhergehenden Ansprüche, dadurch gekennzeichnet, daß das Bindemittel einer Menge von mindestens 25 Gew.% der Trockenbestandteile der Schicht vorhanden ist.
